

June 6, 1944.

J. W. THOMPSON ET AL

2,350,943

COUNTER CURRENT FROTH FLOW FLOTATION SYSTEM

Filed March 2, 1940

4 Sheets-Sheet 1



June 6, 1944.

J. W. THOMPSON ET AL

**2,350,943**

## COUNTER CURRENT FROTH FLOW FLOTATION SYSTEM

Filed March 2, 1940

4 Sheets-Sheet 2



### Inventors:

J.W. THOMPSON  
L.E. BOOTH

By *P.H. Mallinckrodt*  
Attorney

June 6, 1944.

J. W. THOMPSON ET AL

2,350,943

COUNTER CURRENT FROTH FLOTATION SYSTEM

Filed March 2, 1940

4 Sheets-Sheet 3



Inventors:

J. W. THOMPSON  
L. E. BOOTH

By *A. Malindrott.*  
Attorney

June 6, 1944.

J. W. THOMPSON ET AL

2,350,943

COUNTER CURRENT FROTH FLOTATION SYSTEM

Filed March 2, 1940

4 Sheets-Sheet 4



## UNITED STATES PATENT OFFICE

2,350,943

COUNTERCURRENT FROTH FLOW  
FLOTATION SYSTEM

John W. Thompson and Lionel E. Booth, Salt Lake City, Utah, assignors to The Galigher Company, Salt Lake City, Utah, a corporation of Utah

Application March 2, 1940, Serial No. 321,840

11 Claims. (Cl. 209—165)

This invention relates to a countercurrent froth flow flotation system which is advantageously applied to concentration of metallurgical pulps by means of flotation.

The principal objects of the invention are:

First. To produce a higher grade of concentrates by the so-called "rougher" cells of a flotation machine.

Second. To decrease or eliminate the amount of middling return.

Third. To improve the metallurgical efficiency of flotation generally.

Fourth. To increase the metallurgical capacity of flotation machines.

Fifth. To decrease or eliminate the amount of spray or wash water used in launders.

Sixth. To reduce floor space requirements.

Seventh. To allow the direct filtration of flotation concentrates.

Eighth. To simplify the cleaning and re-cleaning operations.

Ninth. In comparison with prior practice, to reduce the quantity of frothing reagent required.

The manner of attaining the objects just outlined, and some of the resulting advantages are set forth briefly in the following paragraphs.

(a) The froth is caused to travel from the tailing end of a flotation machine unit towards the feed end and is discharged in proximity thereto. In the course of its travel from the tailing end to the froth discharge end, the froth drops any gangue or valueless material back into the pulp zone of the machine.

(b) A smaller amount of froth is discharged from the machine and consequently relatively less water and relatively less valueless material are discharged. Advantageously, the middling return is completely or partially eliminated.

(c) Improvement in metallurgical efficiency results because less colloidal or very finely divided valueless material is returned to the head of the flotation unit.

(d) The metallurgical capacity of a flotation machine is increased because of a large decrease in circulating loads and because the spray and launder wash water is virtually eliminated.

(e) Short launders only are required at the point of froth discharge, and as a result, steep slopes can be used, which discharge directly into a pump box or any other convenient point for re-treatment.

(f) The floor space required, is reduced because of increased cell capacity and because of the elimination of side launders for carrying off the froth.

(g) Launders are advantageously placed on steeper grades, thereby allowing for the direct discharge of concentrates to filters.

(h) Rougher froths and intermediate froths are advantageously discharged directly to cleaner

or re-treatment cells without the use of dilution water. This provides for extremely compact installations.

(i) Because less froth is removed from the flotation cells, less frothing reagents are required.

According to the invention, a liquid or semi-liquid such as flotation pulp, is confined as a normally static body. Different parts of the pulp body are subjected to progressively varying bubble generation, for example, by means of aeration or agitation in varying degrees, with the result that correspondingly varying masses of froth containing the valuable mineral of an ore under flotation treatment, are constantly building up on the surface of the pulp. The differences in the levels to which the froth builds up, create potential fluid heads which cause the froth to flow by gravity from the higher levels to the lower levels, and particularly to the lowest level at one end of the pulp body where the froth which carries the finished or partially finished concentrates, is advantageously discharged and saved. The less valuable materials or tailings, on the other hand, are caused to flow counter to the flow of the froth, and are discharged at the other end of the pulp body. This is accomplished by causing the maximum degree of progressive aeration or agitation to take place in proximity to the point of discharge of the tailings.

An advantage of this novel arrangement is that worthless particles or gangue, which may inadvertently be carried up through the pulp by the rising froth, are promptly dropped back into the current of tailings and discarded as waste.

The novel characteristics of the machine of the invention make feasible many original combinations of individual flotation multiple cell units, as will hereinafter be more fully explained. By means of such combinations, large savings in original plant cost, in operating time and expense, and in the cost of reagents may be effected.

Apparatus for practicing the invention may advantageously comprise a plurality of individual flotation cells arranged together in series to form a multiple cell unit in which free communication among the constituent cells, as well as a common pulp level, are maintained, while at the same time, the cells are operatively distinct one from another.

Each cell is advantageously provided with its individual froth generator, and each froth generator is regulable according to the quantity of froth required at its own particular location in the sequence of operations of the multiple cell unit as a whole. The pulp feed is introduced into the first cell, advantageously at a point low in the pulp body, and is conducted successively through the remaining cells of the unit, until

tailings are finally discharged from the last cell.

The froth is made to take a direction of flow opposite to the direction of travel of main body of pulp because an abundance of air is provided with positive control of the quantity of air that is used in each successive flotation cell. Thus the greatest quantity of air is advantageously used at the tailings end of a flotation machine, while progressively smaller quantities of air are used in the successive cells of a series until the first cell at the head end is reached.

The froth containing the valuable minerals of an ore under treatment, progresses from the last cell towards the head end where it is discharged from cell No. 1 in the form of finished or partially finished concentrates, the latter being conducted to a cleaning flotation machine which may or may not utilize the countercurrent froth flow feature.

In the accompanying drawings, which illustrate specific embodiments by means of which the invention is advantageously put into practice,

Fig. 1 represents in plan, a flotation machine comprising for example, four cells;

Fig. 2, a longitudinal, vertical section taken on the line 2—2 in Fig. 1, pipes in the background being omitted;

Fig. 3, a cross-section taken on the line 3—3 in Fig. 2;

Fig. 4, a diagrammatic plan, corresponding to Fig. 1 and serving as a nucleus around which the succeeding Figures 5 to 28 are developed;

Fig. 5, an arrangement similar to Fig. 4, but arranged for producing a better grade of concentrates without middling returns;

Figs. 6 and 7, respectively, a diagrammatic plan and corresponding front elevation showing an arrangement for re-treatment or cleaning of concentrates from multiple cell rougher units;

Figs. 8 and 9, respectively, a diagrammatic plan and corresponding front elevation operatively similar to Figs. 6 and 7, but having the cleaner cells turned through an angle of 90 degrees for straight flow of concentrates over the end of machine for the purpose of economizing floor space;

Figs. 10 and 11, respectively, a diagrammatic plan and corresponding front elevation of an arrangement similar to that in Figs. 8 and 9, but showing the manner in which cells may be added for greater capacity;

Figs. 12 and 13, respectively, diagrammatic plan and corresponding front elevation of an arrangement of cells for double cleaning treatment of metallurgical pulp;

Figs. 14 and 15, respectively, a diagrammatic plan and front elevation showing rougher cells with a drop in elevation between each group of four cells, which facilitates the control and feeding of reagents in certain cases;

Figs. 16 and 17, respectively, a diagrammatic plan and front elevation of a cell arrangement similar to that shown in Figs. 14 and 15, but having the cleaner cells turned through an angle of 90 degrees, for the purpose of giving the concentrates a right line flow through the machine and at the same time accomplishing an economy in floor space;

Figs. 18 and 19, respectively, a diagrammatic plan and front elevation of a cell arrangement having the advantages of operation of those shown in Figs. 16 and 17, but providing for a more compact floor disposition;

Figs. 20 and 21, respectively, a diagrammatic

plan and front elevation of a cell arrangement having operative characteristics similar to those of the arrangement in Figs. 14 and 15, but showing an especially advantageous floor arrangement;

Figs. 22 and 23, respectively, a diagrammatic plan and front elevation of an arrangement having the advantages of that shown in Figs. 14 and 15, but in which the cleaner cells are parallel to the rougher cells, and more cleaner cells are provided for;

Figs. 24 and 25, respectively, a diagrammatic plan and front elevation of an arrangement of rougher cells having a drop in elevation between them as in Figs. 14 and 15, but providing for double cleaning;

Figs. 26 and 27, respectively, a diagrammatic plan and front elevation, of a cell arrangement which accomplishes operative results similar to those accomplished in the arrangement of Figs. 24 and 25, but providing for a considerably more compact floor disposition; and

Fig. 28, an end elevation in diagram, viewed in the direction of the arrow 28 in Fig. 26.

Referring to the drawings, Figs. 1, 2 and 3 show a flotation machine which includes much of the mechanism forming the subject of United States Patents Nos. 2,055,065 and 2,085,947, granted to Lionel E. Booth. This mechanism has novel features which are particularly well adapted for use in combination with the present invention.

Patent No. 2,055,065 is concerned with a rotatable impeller comprising a tight-walled, substantially bell-like structure along the lower circumference of which a plurality of depending teeth or lugs are spaced apart from one another. Compressed fluid, such as air, is conducted into the hollow interior of the bell, and this air is caused to bubble through the spaces between the depending teeth, into the surrounding pulp. The size of the bubbles is determined largely by the speed of rotation of the impeller, while the quantity of bubbles generated is advantageously regulated by the amount of compressed air admitted into the bell.

Patent No. 2,085,947 is concerned with peeling blades that are advantageously disposed radially around the impeller just described, in order to conduct the copious flow of bubbles from the impeller upwardly through the pulp, thereby preventing a congestion of bubbles around the impeller, and thus enhancing the efficiency thereof.

In Figs. 1, 2 and 3, the numeral 40 denotes a structure embracing four successive individual cells 41, 42, 43 and 44, the one at 41 being regarded as the head cell and the one at 44, the tail cell. The pulp is advantageously introduced into head cell 41 through an inlet opening 46 located at the bottom of a feed box 45, the inlet opening being advantageously located low in the cell structure. In this cell, the pulp is exposed to the proper means for producing a certain desired amount of froth which rises through the pulp body 47 and into the space 48—1 above the pulp surface 49. The pulp body is caused to travel successively through the cells 41, 42, 43 and 44 in the general direction of the arrow 53. During the movement of the pulp through the respective cells, it is exposed to a graduated increase in froth generation, which results in a correspondingly greater quantity of bubbles rising through the pulp from cell to cell until the last cell is reached, where the froth production in the present example, is at the maximum. This

results in building a body of froth 48 which is deeper at 48-2 than it is at 48-1, whereby a fluid or hydrostatic head is created approximately along the gradient 50. The froth being extremely mobile, tends to find its fluid surface level because of gravity, and in so doing, a quantity of froth is continually being pushed in the direction of the arrow 54, from the higher froth levels to the lowest froth level, at which latter point it overflows the froth discharge weir 51, to be disposed of as desired.

A hollow, tight-walled impeller is indicated at 56, it being rigidly mounted on a rotatable shaft 57, supported and driven in any suitable manner (not indicated). Spaced apart from one another along the lower circumference of the tight-walled portion 56 of the impeller are depending lugs 55, and projecting upwardly into the interior of the impeller is a pipe 58 through which compressed air is discharged. The compressed air reaches the pipe 58 through the pipe assembly 59 from a main supply header 60, and the flow of compressed air from the header to the impeller may be controlled by a valve 61.

In operation, assuming the impeller to be rotating at the proper speed, which may vary from 1200 to 1900 f. p. m. and assuming the proper amount of compressed air to be flowing into the impeller, the compressed air bubbles through the spaces 62 between the lugs of the impeller. The incipient bubbles are clipped into extremely small bubbles which in rising through the pulp, pick up the mineral and form the froth masses. F. p. m. indicates peripheral feet per minute.

The fine bubbles which are discharged by the impeller are guided upwardly through the froth by means of the peeler blades 63, 64 and 65, it being understood that the number and arrangement of the peeler blades are not restricted by the showing in the present drawing, which represents merely a suggestive arrangement.

The impeller 56 and rotatable shaft 57 are duplicated at 56-1 to 56-3, and 57-1 to 57-3, respectively, in the respective cells 42 to 44. The peeler blades 63 to 65 are also duplicated in the cells 42 to 44, although the duplicates are not shown in the figures.

The amount of froth generated in the successive cells may advantageously be controlled or regulated by precisely varying the relative amounts of compressed air admitted into each respective impeller, by means of valves 61 to 61-3. It is also possible to vary the generation of froth in the successive cells by varying the speeds of rotation of the respective impellers 56 to 56-3.

In order to provide for the free flow of the froth, as well as for the free counterflow of the tailings, it is advantageous to separate the different cells one from another, by comparatively low baffles, such as those indicated at 67 in Figs. 1 and 2. The sidewalls 68 and 69 and endwall 70 serve to confine the froth to the channel formed over the surface of the pulp, and to compel the froth to be discharged at the weir 51, as hereinbefore mentioned. The tailings stream may advantageously be discharged over a weir 71, and disposed of as desired. Both the weirs 51 and 71 may consist of removable flashboards for varying the relative heights thereof.

The multiple cell system of construction is very elastic and adapts itself to an almost endless variety of different circumstances and conditions, so that it becomes possible in any particular case, to achieve the greatest economy of floor space 75

occupied, combined with maximum performance and output of the flotation machine. For the purpose of giving at least a partial understanding of the many combinations of cells that can be advantageously made to meet different requirements, a few of the possible combinations are further illustrated in diagrammatic form in Figs. 5 to 28.

10 The arrangement of cells described in connection with Figs. 1 to 4, produces a good grade of concentrates without middling return, since the froth as it travels along the surface of the pulp from the tailing end of the machine to the concentrate discharge, is cleared of gangue.

15 In Fig. 5, the feed enters at 73, while the tailings and concentrates are discharged at 74 and 75 respectively. This arrangement produces a better grade of concentrates than the arrangement in Fig. 4, also without middling return.

20 The arrangement in Figs. 6 and 7 is one for positive re-treatment or re-cleaning of rougher concentrates. In this arrangement the feed enters at 76 and passes through the four rougher cells 78, discharging the tailings at 79 and the rougher concentrates at 80, from where they pass directly into the cleaner cells 81. The finished concentrates are discharged at 82, while the cleaner tailings are discharged at 83 into a pump 84, from where they are returned into the main 25 feed 85. For convenience, the pump 84 is omitted in Fig. 7.

25 In Figs. 8 and 9 the arrangement is similar to that in Figs. 6 and 7, but the cleaner cells 81-1 have their longitudinal dimensions at right angles to the longitudinal dimension of the rougher cells 78. The pump is indicated at 84-1, and the cleaner concentrates are discharged at 82-1, cleaner tailings at 83-1.

30 In Figs. 10 and 11, the cleaner unit 81-1 is similar to that in Figs. 8 and 9, but the number of individual cells in the rougher unit 86, is increased for greater tonnage. Here, the feed enters at 87. The rougher concentrates are discharged into the cleaner unit at 88, and the rougher tailings are discharged at 89. The cleaner tailings are discharged at 90 and pass into the pump 91 from where they are returned to the feed 87.

35 In Figs. 12 and 13, a double cleaning treatment is provided for. The feed enters at 92, and passes through the rougher unit 93, from which the concentrates pass at 94 into the first cleaner unit 95. The concentrates from the first cleaner unit pass at 96 into the second cleaner unit 97. The tailings from the two cleaner units are discharged at 98 and 99 respectively, and in combination enter the pump 100 which returns them into the feed 92. The finished concentrates from the second cleaner unit are discharged at 101, while the total tailings are discarded from the rougher unit 93 at 102.

40 In Figs. 14 and 15, separate rougher units 103 and 104 are used. Single cleaning is provided for by means of the cleaner unit 105. In this case a drop in elevation between the cells is provided for. This facilitates the control and feeding of reagents in certain cases. The feed enters the first rougher unit 103 at 106, and the concentrates from this unit are discharged at 107 into the cleaner unit 105, while the tailings are discharged at 108, passing into the second rougher unit 104, from where the concentrates are discharged at 111, and the tailings at 112. The tailings from the cleaner unit 105 are discharged at 113 and are passed to the pump 114, being joined meanwhile by the concentrates discharged at 111,

to be returned to the feed at 108. The finished concentrates are discharged at 115.

In Figs. 16 and 17, the arrangement is similar to that in Figs. 14 and 15, with the exception that the cleaner unit occupies the position 105—1, with its longitudinal dimension set at right angles to the longitudinal dimension of the rougher units 103—1 and 104—1.

In Figs. 18 and 19, the arrangement is operationally similar to that in Figs. 16 and 17, but is more compact because the second rougher unit 104—2 is placed in parallel with the first rougher unit 103—2 instead of being in tandem therewith as in Figs. 16 and 17.

In Figs. 20 and 21, the arrangement is operationally similar to that in Figs. 14 and 15, but provides for a different disposition as to floor space. Here, the feed enters the first rougher unit 103—3 at 106—3, while the tailings from the second rougher unit 104—3 are discharged at 112—3. The finished concentrates are discharged at 115—3 from the cleaner unit 105—3.

In Figs. 22 and 23 the general arrangement again is similar to that in Figs. 14 and 15, but more cells are included in the cleaner unit together with a somewhat different floor arrangement. Here, the feed enters at 116 into the first rougher unit 117, the concentrates from which pass at 118 into the cleaner unit 119, while the tailings pass at 120 into the second rougher unit 121. The concentrates from the second rougher unit are discharged at 122, and are joined by the tailings from the cleaner unit which are discharged at 123, the two going to the pump 124 by which they are returned to the feed 116. The total finished concentrates are discharged at 125, and the total tailings are discarded at 126.

In Figs. 24 and 25, the arrangement provides for a drop in elevation between the two rougher units 127 and 128 for the same purpose as that in Figs. 14 and 15, but includes the double cleaning feature by means of two cleaner units 129 and 130. The feed enters at 131; the concentrates from the first rougher unit 127 pass at 132 into the first cleaner unit 129, while the tailings from the first rougher pass at 133 into the second rougher unit 128. The concentrates discharged at 134 from the second rougher, are merged with the tailings discharged at 130—1 and 129—1 respectively from the two cleaner units, and at 135 are pumped back into the feed 131. The total concentrates are discharged at 136 from the first cleaner unit, and the total tailings are discharged at 137 from the second rougher unit.

In Figs. 26 to 28, the arrangement provides for the same general operative result as attained by that in Figs. 24 and 25, but at the same time provides for conservation of floor space. Here, the first rougher unit is indicated at 137, the second at 138, the first cleaner unit at 139, and the second cleaner unit at 140. The feed enters the first rougher at 141, while the concentrates from this rougher enter the first cleaner unit 139 at 142. The tailings from the first rougher enter the second rougher at 143, while the concentrates from the second rougher leave at 144, merge with the tailings from both the cleaner units and are returned by means of the pump 145 to the feed 141. The total finished concentrates are discharged at 146, while the total tailings are discarded at 147. The concentrates from the first cleaner 139 go through the passage 148 into the second cleaner 140 and the tailings from the second cleaner are discharged at 149.

The structure illustrated in Figs. 1 to 4, may

be described as composed of the individual cells 41 to 44, or it may consistently be regarded as embracing only a single cell whose configuration is longitudinally extensive and which is provided with means for quantitatively graduated froth generation from end to end, or in which froth generators are spaced apart from one another along the longitudinal dimension with means for precisely varying the production of froth by the successive generators. If desired, the baffles 67 may sometimes be omitted, which still further emphasizes the single cell viewpoint.

In any event, the distinguishing feature of the machine is always the open and substantially unobstructed passage for pulp and froth in counter-current relation to each other from end to end of the structure. This viewpoint applies to the various assemblies of units shown in Figs. 5 to 28, as well as to the unit shown in Figs. 1 to 4. For example, the assembly as shown in Figs. 12 and 13, consists of the three units 93, 95 and 97, where the passage through the rougher unit 93 is open and unobstructed from the end 151 to the other end 152, although including six individual impeller spaces each provided with its own impeller 153.

Again, in the same figures, the open passage through the first cleaner unit 95 extends from the end 154 to the other end 155, and in the second cleaner unit 97, from the end 156 to the other end 157.

Another example is the assembly in Figs. 26 to 28. Here the open passage through the first rougher 137 extends between the ends 158 and 159; the open passage through the second rougher 138, between the ends 160 and 161; the open passage through the first cleaner 139, between the ends 162 and 163; and through the second cleaner 140, between the ends 164 and 165.

In the most advantageous form of the machine, the two sidewalls, such as 68 and 69 in Figs. 1 and 2, are sufficiently high so that the froth is prevented from overflowing excepting at the end weir 51. There are times however, when it becomes desirable to discharge the froth over either one or both sidewalls. In such cases these walls are provided with removable flashboards, for example, such as those shown at 170, 171, 172 and 173. When these flashboards are removed, the froth may overflow at suitably graduated levels, for example, those represented by the bottom edges of the flashboards, which in this instance follow closely the gradient 50. By removing such flashboards in various combinations thereof, almost any desired control may be exercised over the sidewall froth discharge. The sidewall discharge of froth may be carried off by any suitable means, for example, by launders 174.

The invention is characterized by the counter-current relationship existing between the froth flow and the flow of the at-least-partially-im-poverished pulp or tailings, as hereinbefore explained. It should be remembered however, that while the froth flow in this relationship is along the substantially level surface of the pulp body, the counterflow of the pulp and its suspended tailings is not likewise substantially horizontal. In fact, it is only the net transportative displacement of the pulp and its tailings that is horizontal, because both are subjected to the varying upwardly directed impulses in the successive bubble column zones. This variation causes many of the pulp particles, including tailings, to circulate upwardly and downwardly during the progress of this horizontal displacement.

In the present instance, horizontal displacement is imparted to the body of pulp and to the tailings which are suspended therein, by means of the incoming feed at 46 which tends, as usual, to create a slight hydrostatic head of the pulp body, and therefore to cause the overflow of the at-least-partially-impoverished pulp at discharge weir 71. Aerating or agitating the pulp assists in its horizontal displacement, since the air-impregnated pulp occupies more space than does the normal pulp body, thus increasing the overflow at the weir 71 accordingly.

The aerating mechanism of the aforementioned Patent 2,085,947 is especially well suited for use in combination with the present invention, because air or other fluid is admitted to the impeller under pressure, usually from three-fourths to one and one-half pounds per square inch. The flow of this compressed fluid through each successive impeller, is subject to accurate control, whereby the requirements of the invention for precisely differentiated generation of fluid bubbles to form froth in differential quantities at the corresponding localities on the surface of a pulp body, are fully accomplished.

It is the ability to control the constant formation of froth at definite points and in certain predetermined quantities that makes possible the gravity flow of the froth across the surface of a pulp body in opposition to the movement of the pulp body, which in this instance is in the direction of the weir 71, and occasioned by the overflow at that point.

In ordinary flotation, froth is removed along the full length of a machine. Since large proportions of the reagents used, are removed with the froth, the frothing properties towards the tail end of a machine are materially diminished, frequently to a point where it is difficult to maintain a froth overflow at all at this end of the machine.

In using the countercurrent flow feature, it is to be noted that since the froth breaks down in traveling from the tail end to the head end, water composing the bubbles, together with reagents, is dropped back into the pulp body and is again carried towards the tail end of the machine, thus using this part of reagents over and over again.

Performance of the countercurrent froth flow system compared with performance of what has heretofore been regarded as standard practice, in actual operating tests, gave results as follows:

*Test No. 1*

|                                           | Zn              | Fe             | Insol.         |
|-------------------------------------------|-----------------|----------------|----------------|
| C. C. F. F. system:                       |                 |                |                |
| Concentrates.....                         | Percent<br>63.0 | Percent<br>0.8 | Percent<br>2.1 |
| Tailing.....                              | 1.3             |                |                |
| Standard practice at Silver King<br>Mill: |                 |                |                |
| Concentrates.....                         | 63.2            | 0.8            | 1.3            |
| Tailing.....                              | 1.6             |                |                |

*Test No. 2*

|                                           | Zn              | Fe             | Insol.         |
|-------------------------------------------|-----------------|----------------|----------------|
| C. C. F. F. system:                       |                 |                |                |
| Concentrates.....                         | Percent<br>62.6 | Percent<br>0.7 | Percent<br>2.0 |
| Tailing.....                              | 1.1             |                |                |
| Standard practice at Silver King<br>Mill: |                 |                |                |
| Concentrates.....                         | 63.0            | 0.8            | 1.6            |
| Tailing.....                              | 1.0             |                |                |

It will be noticed that the concentrate recov-

eries and tailing losses are practically the same for both the countercurrent froth flow tests and the Silver King tests. The Silver King Mill uses triple cleaning, in other words, the rougher concentrates are re-treated three times in order to produce its concentrates. In contrast to this, the concentrates produced by the countercurrent froth flow system as above indicated, are the result of a single operation. The operating advantages in reduced number of machines to accomplish equivalent results, and corresponding savings in first cost of equipment, together with material savings in power costs and savings in maintenance expenses, in favor of the system of the invention, are self evident. The direct savings in reagents hereinbefore dwelt upon, are in addition to the savings just enumerated.

Having fully described our invention what we claim is:

1. A method of counter-current froth-flow flotation, comprising feeding flotation pulp substantially constantly into one end of a normally static, longitudinally extended body of flotation pulp which has substantially uniform width, thereby imparting a substantially constant, and substantially unidirectional, longitudinal displacement or transition to the pulp body and causing pulp to discharge at the opposite end of the pulp body; introducing air into the transient pulp body in graduated quantities from end to end thereof, the greatest quantity being introduced at the said pulp discharge end; and accumulating the resulting bubbles in the form of froth on the surface of the pulp body substantially in the proportion of air introduction at corresponding points along the length of the pulp body, thereby forming a hydrostatic head of froth, and causing the said froth to flow by gravity along the surface of the pulp body counter to the direction of transition of the pulp, by confining the said froth against discharge at said pulp discharge end and laterally along the length of the pulp body.
2. A method of counter-current froth-flow flotation, comprising feeding flotation pulp into one end of a normally static, longitudinally extended body of flotation pulp which has substantially uniform width, thereby imparting a substantially constant, substantially unidirectional, longitudinal displacement or transition to the pulp body and causing pulp to discharge at the opposite end of the pulp body; conducting the transient pulp through a plurality of longitudinally aligned froth generating zones which merge at least partially one into another, the said froth generating zones extending from near the locality of feeding pulp to near the locality of discharging pulp; generating froth in the successive generating zones with increasing intensity of generation from zone to zone, the least intensity being in proximity to the locality of feeding pulp, and the greatest in proximity to the locality of discharging pulp, thereby causing froth to rise to the surface of the pulp body in quantities which are substantially proportional to the successive intensities of generation; and accumulating the said froth on the surface of the pulp body as it rises, thereby forming a hydrostatic head of froth, and causing said froth to flow by gravity along the surface of the pulp body counter to the direction of transition of the pulp, by confining the said froth against discharge at the locality of discharging pulp and laterally along the length of the pulp body substantially up to the vicinity of said locality of feeding pulp.

3. A method of counter-current froth-flow flotation, comprising maintaining a longitudinally extended body of flotation pulp having substantially uniform width; introducing air into the lower portion of the pulp body in successively graduated quantities from maximum to minimum along the length thereof and within an aerating zone which is substantially coextensive horizontally with the said pulp body, to form bubbles which rise through the pulp body and to the surface thereof in substantially correspondingly graduated quantities; continuously supplying additional pulp to the pulp body near one end thereof and continuously discharging tailings near the opposite end thereof, thereby causing the aerated pulp to flow in a substantially continuous, substantially unidirectional longitudinal stream from the pulp inflow end of the pulp body to the tailings discharge end thereof and immediately above said aerating zone; accumulating the bubbles in the form of froth at the surface of the pulp body substantially in the proportion of air introduction at corresponding points along the length of the pulp body, thereby forming a hydrostatic head of froth, and causing the said froth to flow by gravity along the surface of the pulp body counter to the direction of transition of the pulp, by confining the said froth against discharge at said tailings discharge end and laterally along the length of the pulp body; and discharging said froth from the surface of the pulp body near said pulp inflow end thereof.

4. A method, as recited in claim 3, wherein a minor part of the froth is discharged at a locality or localities situated between the two end extremities of the pulp body.

5. A flotation machine, comprising an elongated container adapted to hold a body of pulp; aeration means disposed in an aerating zone defined at a low level within said container and said means extending along the length thereof; pulp inflow means disposed near one end of said container; tailings outflow means disposed near the opposite end of said container; froth outflow means disposed at the upper part of said container near said pulp inflow means; and means for effecting flow of froth along the surface of said body of pulp substantially from the tailings-outflow end of said container to the said froth discharge means, said container having its interior, above said aerating zone, substantially free and unobstructed so pulp may flow substantially horizontally, substantially unidirectionally, and longitudinally, from said pulp inflow means to said tailings outflow means and within a zone disposed above said aerating zone.

6. A flotation machine, comprising an elongated container having substantially uniform width and adapted to hold a body of pulp; aeration means disposed in an aerating zone defined at a low level within said container and said means extending along the length thereof; pulp inflow means disposed near one end of said container; tailings outflow means disposed near the opposite end of said container; froth outflow means disposed at the upper part of said container near said pulp inflow means; and means for regulating the supply of air to said aeration means so that said supply of air will be a maximum near the tailings-outflow end of said container and a minimum near the pulp-inflow end of said container, resulting in the building up of a hydrostatic head of froth upon the surface of the body of pulp at the tailings-outflow end

of said container, and in the gravity flow of froth from said tailings-outflow end to said pulp-inflow end of the container during operation of said flotation machine, said container having its interior, above said aerating zone, substantially free and unobstructed so pulp may flow substantially horizontally, substantially unidirectionally, and longitudinally, from said pulp-inflow means to said tailings-outflow means and within a zone disposed above said aerating zone.

7. A flotation machine, comprising an elongated container adapted to hold a body of pulp, said container having its lower portion partitioned off at intervals along its length transversely of its width forming individual aeration cells; mechanical aerating means disposed in the respective aeration cells; pulp inflow means disposed near one end of said container; tailings outflow means disposed near the opposite end of said container; froth outflow means disposed at the upper part of said container near said pulp inflow means; and means for effecting flow of froth along the surface of said body of pulp substantially from the tailings outflow end of said container to the said froth discharge means, said container having its interior, above said aeration cells, substantially free and unobstructed so pulp may flow substantially horizontally, substantially unidirectionally, and longitudinally, from said pulp inflow means to said tailings outflow means and within a zone disposed above said aeration cells.

8. A flotation machine, comprising an elongated container having substantially uniform width and adapted to hold a body of pulp; said container having its lower portion partitioned off at intervals along its length transversely of its width forming individual aeration cells; mechanical aerating means disposed in the respective aeration cells; pulp inflow means disposed near one end of said container; tailings outflow means disposed near the opposite end of said container; and means for regulating the extent of aeration within the respective aeration cells so that the aeration will be a maximum near the tailings outflow end of said container and a minimum near the pulp-inflow end of said container, resulting in the building up of a hydrostatic head of froth upon the surface of the body of pulp at the tailings outflow end of said container and in the gravity flow of froth from said tailings outflow end to said pulp inflow end of the container during operation of said flotation machine, said container having its interior, above said aeration cells, substantially free and unobstructed so pulp may flow substantially horizontally, substantially unidirectionally, and longitudinally, from said pulp inflow means to said tailings outflow means and within a zone disposed above said aeration cells.

9. In a flotation system, a plurality of flotation units interconnected in series arrangement to effect a single final discharge of froth, each of said flotation units comprising an elongated container for pulp having substantially uniform width and defining along its length a lower aeration zone, an intermediate separation zone, and an upper froth transportation zone, the said separation zone and froth transportation zone extending substantially free and unobstructed along substantially the entire length of the said container, the container having pulp inflow means and froth outflow means near one of its ends, and tailings outflow means near its opposite

end, and having further, means for aerating pulp differentially substantially from end to end of said aeration zone, the locality of greatest aeration being near the tailings outflow end of the container, and the locality of least aeration being near the pulp inflow end thereof, resulting in the building up of a hydrostatic head of froth upon the pulp body and within said froth transportation zone during operation of said system, whereby froth flows along said froth transportation zone toward said froth outflow means under the influence of gravity, and pulp flows substantially unidirectionally counter thereto; and respective passage means connecting the said froth outflow means of each of the said flotation units, except the last, with the said pulp inflow means of the next succeeding.

10. A method of countercurrent flotation comprising, maintaining a longitudinally extended body of flotation pulp; introducing air into the lower portion of the pulp body, within an aerating zone which is substantially coextensive horizontally with the said pulp body, to form froth which rises through the pulp body and accumulates at the surface thereof; continuously supplying additional pulp to the pulp body near one end thereof, and continuously discharging tailings from the pulp body near the opposite end thereof, thereby causing the aerated pulp to flow in a substantially continuous, substantially unidirectional, longitudinal stream from the pulp inflow end of the pulp body to the tailings discharge

5 end thereof and immediately above said aerating zone; flowing the said accumulated froth on the surface of the pulp body and along the length thereof from near said tailings discharge end of the pulp body toward the said pulp inflow end thereof; and discharging said froth from the surface of the pulp body near said pulp inflow end thereof.

11. In a flotation system, a plurality of flotation units interconnected in series arrangement to effect a single final discharge of froth, each of said flotation units comprising an elongated container for pulp defining along its length a lower aeration zone, an intermediate separation zone, and an upper froth transportation zone, the said separation zone and froth transportation zone extending substantially free and unobstructed along substantially the entire length of the said container, the container having pulp inflow means and froth outflow means near one of its ends and tailings outflow means near its opposite end, so that pulp flows in a substantially unidirectional, longitudinal stream, and having, further, means for flowing froth along said froth transportation zone, counter to the said flow of pulp, and out of said froth outflow means; and respective passage means connecting the said froth outflow means of each of the said flotation units, except the last, with the said pulp inflow means of the next succeeding.

JOHN W. THOMPSON.  
LIONEL E. BOOTH.